

# UNITED STATES PATENT OFFICE.

HENRY K. SANDELL, OF CHICAGO, ILLINOIS, ASSIGNOR TO HERBERT S. MILLS, OF CHICAGO, ILLINOIS.

## ALLOY BEARING.

1,223,001.

Specification of Letters Patent. Patented Apr. 17, 1917.

No Drawing.

Application filed June 19, 1916. Serial No. 104,453.

*To all whom it may concern:*

Be it known that I, HENRY K. SANDELL, a citizen of the United States, residing at Chicago, in the county of Cook and State 5 of Illinois, have invented a new and useful Improvement in Alloy Bearings, of which the following is a specification.

My invention relates to certain improvements in journals, or bearings. More particularly, the invention is concerned with a metallic alloy which is peculiarly advantageous in such uses, exhibiting as it does in actual practice the properties of low frictional resistance and long life.

15 The alloy in question consists of copper and antimony, in substantially the proportion of two parts (by weight) of the former, to one part of the latter, together with a smaller proportion of lead, and preferably 20 in addition thereto a percentage of nickel.

For example, I find that for use as a bearing-bushing for supporting the steel shaft of a 10 K. W. dynamo electro machine turning about 1800 R. P. M., the following composition is desirable.

|                |   |
|----------------|---|
| Copper -----   | 4 |
| Antimony ----- | 2 |
| Lead -----     | 1 |
| Nickel -----   | 1 |

In general, it appears that the antimony possesses the property of crystallizing the copper, thereby greatly increasing the hardness of the compound and lowering the frictional resistance.

The nickel is desirable as tending to toughen the alloy; that is, bind together the highly crystalline mass, increase its tensile strength and prevent disintegration under abrasive action. The lead appears to be to 40 some extent useful as a toughener, but I believe that its main value is probably akin to that of a lubricant.

A bearing cast from an alloy of the metals mentioned is capable of running for 45 an indefinite period without lubrication, and without showing substantial wear. It displays no tendency to overheat, does not itself score, nor score its shaft, and is in all respects satisfactory for use as a bearing-bushing operating under sliding friction, either entirely without lubrication, or with 50 very little lubrication at moderate bearing pressures and high speeds.

What I claim as new, and desire to secure 55 by Letters Patent, is:

1. A bearing comprising substantially fifty per cent. of copper, twenty-five per cent. of antimony and proportionate amounts of lead and nickel. 60

2. A bearing formed of an alloy comprising relatively large proportions of copper, antimony and an additional constituent which will increase the tensile strength.

3. A bearing formed of an alloy consisting of four parts (by weight) of copper, two parts of antimony, one part of nickel, and one part of lead. 65

HENRY K. SANDELL.